

May 27, 1969

P. ESSLINGER ET AL

3,445,920

## ALUMINUM BASE ALLOY PRODUCTION

Filed May 5, 1966

Sheet 1 of 3



Fig. 1

May 27, 1969

P. ESSLINGER ET AL

3,445,920

ALUMINUM BASE ALLOY PRODUCTION

Filed May 5, 1966

Sheet 2 of 3



A: 6% Mn, 8% Fe, BALANCE Al, PREPARED ACCORDING  
TO INVENTION

B: 5.5% Zn, 2.8% Mg, 0.5% Mn,  
0.4% Cu, BALANCE Al  
C: 6.0% Cu, 0.25% Mn, 0.1% Ti  
BALANCE Al } CONVENTIONALLY  
PREPARED

FIG.2

May 27, 1969

P. ESSLINGER ET AL

3,445,920

ALUMINUM BASE ALLOY PRODUCTION

Filed May 5, 1966

Sheet 3 of 3



I. CAST ACCORDING TO INVENTION  
2. CONVENTIONALLY CAST

FIG.3

1

3,445,920

ALUMINUM BASE ALLOY PRODUCTION  
Paul Esslinger, Stuttgart, Heinrich Winter, Eschborn  
Taunus, and Walter Wolf, Frankfurt am Main, Germany, assignors to the Federal Republic of Germany as  
represented by the Secretary of Defense, Bonn, Germany

Filed May 5, 1966, Ser. No. 547,939

Claims priority, application Germany, May 11, 1965,  
B 81,85410 Int. Cl. C21d 7/14; B22d 19/00  
U.S. Cl. 29—472.3

4 Claims

## ABSTRACT OF THE DISCLOSURE

An aluminum base alloy is produced by melting the alloy and passing it between closely spaced cooling and forming surfaces which compact the molten alloy into a thin sheet having a thickness of 1 mm. or less.

This invention relates to a method for producing ductile aluminum alloys of high strength at elevated temperatures.

It is known that the strength of metals at room temperature and elevated temperatures can be increased by suitable alloying additions. However, in malleable alloys, the amount of such additives cannot, at present, be increased at will unless the alloying additive gives with the base metal an extensive area of mixed crystal formation in the solid state.

When the amount of alloying additive exceeds the maximum solubility in the solid state, there are formed in the structure of the material inclusions of generally brittle and sharp edged intermediary phases which can no longer be eliminated by a solution heat treatment. The number and particularly the size of said phases increase with increased amounts of the alloying additive. They render the alloy brittle, and it is generally sufficient to exceed the solubility by a few percents to prevent useful deformation, particularly cold working of the alloy. The inclusions do not, or hardly, contribute to the strength of the alloy because, in normal production, their size is in excess of 1  $\mu\text{m}$ . Particles of such size are not able of hindering substantially the slippage inside the material in plastic deformation. Instead, they act mostly as nuclei for the formation of internal cracks.

It is also known to prepare structures having finely distributed inclusions by applying high cooling rates. In order to obtain a reasonable increase of strength, the inclusions must be very small and have an order of magnitude of 0.01 to 1  $\mu\text{m}$ .

In order to obtain dispersions of such fine particles, the cooling rate of the dispersions during casting must be extremely increased, to an order of magnitude of  $10^3$  to  $10^4$   $\text{C/sec.}$  and higher. At such cooling rates, other known effects take place, such as precipitation of metastable phases in fine dispersions and extension of the area of mixed crystallization; both effects can considerably increase the strength, particularly the high temperature strength.

Heretofore, it has not been possible to make use of this knowledge because the recited rapid cooling rates could be realized only at castings having a wall strength of less than 1 mm.

Such thin castings cannot be prepared with conventional casting procedures. In addition, cooling rates of such order of magnitude were difficult to obtain because at beginning solidification the casting shrinks and an air gap is formed between the casting and mold, which interrupts the heat contact.

A sufficiently high cooling rate is obtained in the

2

known atomization of melts. The thus obtained powder is then compacted; in this way, special aluminum alloys of good elevated temperature properties can be obtained. However, this method presents the following drawbacks:

5 The powder metallurgical processing is relatively complicated and increases the cost of the alloy. In addition, heat treatments are required at rather high temperatures, which in many alloys destroy the favorable structures. Thereby, oxide and oxide hydrate inclusions are unavoidable whose sizes, forms, and quantities cannot be controlled.

On heating, the oxide hydrates give off water which can react with the metallic components to form hydrogen. 15 The oxide inclusions as well as the hydrogen reduce the ductility of the alloys.

Said drawbacks are avoided according to the invention by melting an aluminum alloy, preferably without a crucible, by cooling the melt rapidly between at least two 20 moving cooling bodies, and by forming the melt simultaneously to thin bodies, e.g., films, of a thickness of about 1, preferably 0.1 to 0.5 mm. The thus obtained alloys having high ductility and high strength at elevated temperatures; the alloying elements are segregated from 25 stable or metastable phases as finely dispersed particles having a diameter of 0.1 to 1  $\mu\text{m}$ , or are dissolved in metastable form.

Thin shaped articles made in accordance with the method of the invention from alloys which have a high 30 proportion of brittle intermediary phases and which remain brittle in conventional casting methods are readily cold-worked without affecting their strength and ductility. Such aluminum alloys are, e.g., Al-Mn alloys containing up to 9% by weight of manganese, Al-Cr with up to 6% 35 by weight of chrome, Al-Cr-Si and Al-Mn-Si alloys containing up to 20% of the alloying additives, and others.

According to a further embodiment of the invention, semifinished articles and workpieces of greater thickness can be made from alloys by compacting a plurality of 40 said thin shapes to packs by rolling or pressing, particularly at moderately elevated temperatures (press welding) to the desired end product. For Al-Si alloys, for instance, a suitable temperature is about 300° C. Such procedure is possible because the thin shapes obtained 45 by our method have a surprising workability which is far beyond the usual workability.

Our novel method offers the possibility to prepare finished and semifinished articles, such as sheets, strips, and sections by deformation from alloys which heretofore in conventional casting methods were obtained so brittle as not to allow further working by technical deformation. This presents a considerable advance because the alloys prepared in accordance with the invention have a particularly advantageous fine structure and at 55 the same time a surprisingly high strength, even at elevated temperatures.

When applying the method of the invention to heterogeneous alloys of conventional composition, their strength, workability and recrystallization temperature are considerably increased; this is of advantage particularly for the use of such alloys at elevated temperatures.

The invention will be described in more detail with reference to the accompanying drawings wherein:

FIG. 1 shows an apparatus suitable for carrying out 60 the method of the invention;

FIG. 2 shows the variation of the tensile strength as a function of the temperature for alloys made in accordance with the invention in comparison to conventionally compared alloys, and

70 FIG. 3 is a diagram similar to FIG. 2, showing the variation of the tensile strength as a function of the tempering temperature.

Referring now first to FIG. 1, the reference numeral 1 represents a suitably wound induction coil in which the alloy 2 can be molten in free-floating condition. Any other suitable melting procedure can be employed, e.g., a so-called self-consuming electrode can be molten continuously by means of an electric arc or electron beam. The molten alloy passes into the cooling device 3 which consists of at least two movable cooling bodies of high heat conductivity (e.g. copper or silver). In the example, said cooling bodies have the form of movable plates which can be displaced rapidly against each other so as to form therebetween, with simultaneous uninterrupted cooling, the melt to thin bodies, e.g. films of at most 1 mm. thickness. Thereby, said plates act as molds following the shrinkage of the solidifying metal. A similar effect can be also accomplished, for example, by employing as cooling bodies rotating cylinders.

In the embodiment illustrated in the drawing, the cooling elements are actuated by the solenoids 4, which are switched on by the melt itself on its travel into the molds by means of the photoelectric cell 5. Said cell 5 is electrically connected to the solenoid 4 by means of a control device 6, which operates with a predetermined delay. By adjusting said delay with respect to the distance between photoelectric cell and cooling elements, we ensure that said cooling elements move quickly towards each other at the right moment.

The thickness of the films and e.g. also of wires can be adjusted by suitable control of the melting temperature, the rate of movement and pressure of the cooling elements and their distance, to the range of 0.1 to at most 1 mm.

The following examples are given to illustrate the invention.

#### Example 1

An aluminum base alloy having the composition 6% by weight manganese, 8% by weight iron, balance aluminum, was cast in conventional manner in a copper chill mold to round bars of 10 mm. diameter. On the other hand, the same alloy was used to prepare films of about 0.3 mm. thickness in accordance with the invention. While the conventionally cast rods were extremely brittle at elevated temperatures already at the slightest deformation, the films could be cold rolled by about 50% without any difficulties. In the cold rolled state, they gave the values of cold and heat resistance shown in the hatched range A of FIG. 2. The curves B and C show the corresponding values of conventional aluminum alloys having comparable strength at low temperatures.

#### Example 2

Specimens were prepared from eutectic aluminum-silicon casting alloys, on the one hand, in conventional manner in sand or chill molds, and, on the other hand, as films by the process of the invention. The specimens were cold rolled and tested for their tensile strength at room temperature after tempering for 1 hour at the various temperatures indicated as abscissae in FIG. 3.

The dotted line shows the values measured on conventionally cast alloys. The full line shows the tensile

strength for specimens of the same alloy produced according to the invention.

The diagram shows that the method of the invention almost doubles the tensile strength and raises the recrystallization temperature by about 100° C. In addition, the alloy made according to the invention had considerably better workability.

#### Example 3

Aluminum base alloys containing about 3% iron and 3% silicon, when cast by conventional methods, are workable only with difficulty. In contrast thereto, films or foils made by the method of the invention offer a workability and deformability which are far superior to the properties attainable heretofore.

#### Example 4

For the manufacture of bolts having a diameter of 10 mm., as used for the production of heat resistant screws, discs of a diameter of 50 mm. were punched from a sheet of 0.3 mm. thickness of an Al-Mn-Fe alloy obtained by the process of Example 1. 300 such discs were packed upon each other and compressed in an extrusion press at a pressure of 1500 atm. and at a temperature of 350° C. to the article. The high temperature tensile strength of the bolts was much higher than that of bolts made from the same alloy by conventional casting.

We claim:

1. A method of producing an aluminum base alloy having good ductility and high strength at elevated temperatures comprising passing a free-flowing melt of an aluminum base alloy through a narrow gap defined by cooling surfaces spaced from each other by not more than about 1 mm., solidifying the alloy in said gap, the sudden cooling in said gap precipitating the alloy elements in said alloy substantially as finely dispersed particles having a diameter of 0.1 to 1  $\mu$ m., and compressing the alloy, while being solidified, on its passage through said gap to a sheet of a thickness of at most 1 mm.

2. The method as claimed in claim 1 wherein the width of said gap at its narrowest point is 0.1 to 0.5 mm.

3. The method as claimed in claim 1 including the step of joining said sheets to articles of greater thickness.

4. The method as claimed in claim 3 superposing a plurality of said sheets and uniting the same at elevated temperatures.

#### References Cited

##### UNITED STATES PATENTS

|           |         |                |          |
|-----------|---------|----------------|----------|
| 2,967,351 | 1/1961  | Roberts et al. | 29—420.5 |
| 3,147,521 | 9/1964  | Boehm          | 29—528 X |
| 3,214,805 | 11/1965 | McKenica       | 164—75 X |
| 3,368,273 | 2/1968  | Maltsev et al. | 29—528   |
| 3,374,826 | 3/1968  | Black          | 29—528 X |

55 JOHN F. CAMPBELL, *Primary Examiner*.

P. M. COHEN, *Assistant Examiner*.

U.S. Cl. X.R.

60 164—75; 148—2